

Aug. 13, 1935.

E. M. MAY

2,011,007

METHOD OF MAKING COMPOSITE VALVES

Original Filed Oct. 23, 1931 2 Sheets-Sheet 1



FIG. 1.



FIG. 2.

INVENTOR:

Edward M. May  
By  
Ray J. Gehr

ATTORNEY.

Aug. 13, 1935.

E. M. MAY

2,011,007

METHOD OF MAKING COMPOSITE VALVES

Original Filed Oct. 23, 1931 2 Sheets-Sheet 2



FIG. 3.



FIG. 4.



FIG. 5.

INVENTOR:  
Edward M. May  
By  
Ray S. Gehr  
ATTORNEY

## UNITED STATES PATENT OFFICE

2,011,007

## METHOD OF MAKING COMPOSITE VALVES

Edward M. May, Detroit, Mich.

Original application October 23, 1931, Serial No. 570,647. Divided and this application October 13, 1933, Serial No. 693,481

12 Claims. (Cl. 29—157.1)

The invention relates to the production of composite valves and especially valves having seat-engaging parts formed of very hard wear-resisting metal, the present application being a division of my copending application Serial No. 570,647, filed October 23, 1931.

For various uses valves are required which are capable of prolonged use without sufficient deterioration from mechanical wear or corrosion to impair their effectiveness. This is especially true of uses in which the working conditions are such as to make renewal of a valve difficult and a thing to be avoided if possible. The known metals which have the requisite durability to meet these requirements are exceedingly hard and, in some cases at least, cannot be forged or finished by machining but must be formed by casting and finished by grinding. Furthermore, such metals, or at least some of them, tend when cast, especially when cast in metal molds and rapidly chilled, to have a porous interior structure and this makes it difficult to secure smoothly finished seat-engaging surfaces when it is necessary to grind away the outer metal of the casting. The alloy stellite is an example of such metals, it being particularly suitable, because of its great hardness and ability to resist wear and corrosion, to form the seat-engaging part of a valve of the character in question.

The nature of the method and the manner in which it is carried out will most readily be understood from a consideration of specific valve constructions and of apparatus suitable for the carrying out of the method. In the accompanying drawings I have illustrated two forms of valve construction by way of example and mold apparatus such as I prefer to employ.

While my improved method, at least in some of its aspects, is adapted to the production of various forms of valves, it is, in certain respects, particularly applicable to needle valves which may have an elongated shank part of steel or other suitable metal and a tip or head part formed of metal having great hardness and the ability to strongly resist wear and corrosion. Accordingly I shall explain and describe my improved method in connection with the production of needle valves of this character.

One of the chief objects of the present invention is the provision of a method of producing composite valves of the character referred to in which difficulties incident to the porosity of the cast part of the valve structure are effectively overcome.

Another object of the invention is the provision of a method of producing a composite valve in which the different parts of the valve are effectively united to form a rigid unit.

A further object of the invention is the provision of a method of producing composite valves

of the character in question in which the labor required and the loss of materials resulting from defectives or otherwise are minimized, with resultant lowering of the cost of production.

Other objects more or less incidental or ancillary to those above stated, as well as preferred ways of attaining the objects, will be apparent from the following description.

In the drawings, Fig. 1 is a plan view of one form of mold with parts thereof broken away to show interior construction.

Fig. 2 is a view, partly in side elevation and partly in vertical axial section, of the mold shown in Fig. 1.

Fig. 3 is a view of the same character as Fig. 2 showing a modified form of mold.

Fig. 4 is a side view, partly in axial section, of a valve produced by my improved process.

Fig. 5 is a similar view of a modified form of valve construction produced by a somewhat modified form of the method employed in producing the valve in Fig. 4.

Referring first to the valve construction shown in finished form in Fig. 4, and disregarding the dot-and-dash lines of said figure which have to do with the method of manufacture, said valve comprises a shank 1 formed of steel or other suitable metal having physical characteristics adapting it to be readily machined and to perform suitably the usual functions of a valve shank. If the contemplated use of the valve is such as to call for high resistance to corrosion, I prefer to make the shank of a metal such as stainless steel. The shank 1 is machined at one end to form an axially extending cavity, the walls of which are undercut at the inner end of the cavity to form a taper shoulder 2 and are beveled at the outer end of the cavity to form an oppositely inclined taper shoulder 3. The outer surface of the shank at the same end is formed with an outer taper or bevel 4.

To the end of the shank 1 is secured a seat-engaging tip 5 of suitable hard, wear-resisting metal such, for example, as stellite. As is well known, stellite is both exceedingly hard and highly resistant to corrosion. Because of its hardness it cannot be rolled or forged but must be formed by casting and, for the same reason, it cannot be machined but must be finished by grinding. Accordingly I secure the tip to the shank by casting it on the end thereof, the molten metal of the casting entering the cavity in the end of the shank and forming, when the metal sets, an interlocking connection between the two parts. That is, the enlarged inner end or knob 5a of the tip 5 is formed with an annular taper 6 which engages the opposing taper 2 of the shank and the outer part of the tip is formed with an annular taper 7 which similarly engages the opposing taper 3 of the shank. The crys-

- tallization and temperature shrinkage of the metal of the stem 5<sup>b</sup> of the tip on setting and cooling causes the tapered shoulders 6 and 7 thereof to be drawn very strongly against the 5 opposing shoulders 2 and 3 of the shank so as to secure the tip and shank rigidly together. The contraction of the metal of the tip leaves small voids or clearances at the inner end of the tip and around the periphery thereof as shown 10 in Fig. 4, but the firm engagement of the taper shoulders of the tip and shank very effectively holds the two parts rigidly together. In the drawings the size of the voids is exaggerated for the sake of clearness.
- 15 The shank 1 of the valve may, if desired, be formed with a hole as at 1<sup>a</sup> to receive a securing screw or pin.

I shall now describe the mold apparatus shown in Figs. 1 and 2 and the manner of using it in carrying out my improved method of producing composite valves. The specific mold construction illustrated is designed for the simultaneous casting of a considerable number of valve tips or heads of valves of the character shown in Fig. 4 20 and the mold is adapted to employ centrifugal force for feeding the molten metal into the mold cavity. The mold body comprises a circular bottom part 8 and a similarly shaped top part 9 which is secured to the bottom part by a plurality 25 of stud bolts 10 and nuts 11. I have found mee-hanite a suitable material for the main mold parts 8 and 9, the same being a cast metal with properties between those of cast iron and cast steel. The stud bolts are secured rigidly in 30 threaded holes in the bottom part and extend through plain holes in the top part so that the top part of the mold can readily be lifted off when the nuts 11 are removed. To provide for the rotation of the mold, the bottom part 8 is 35 formed with a depending hub 8<sup>a</sup> which is drilled out to fit the upper end of an upright drive shaft 12 to which the hub is detachably secured by a set screw 8<sup>b</sup>. In the construction shown, this 40 shaft is the upwardly projecting end of the armature shaft of an electric motor 13.

The upper part 9 of the mold is formed with a relatively large central opening 14 which, in conjunction with the upper face of the lower part 8, forms the pouring cavity of the mold. 45 The opening 14 preferably has its side wall undercut as shown in Fig. 2. Surrounding the opening 14 are a circumferential series of cavities 15, 15 to receive valve shanks and, in conjunction with the shanks, form a corresponding number 50 of casting cavities for the valve tips. These mold cavities extend radially and are formed by mating depressions in the opposing faces of the lower and upper parts of the mold. Each cavity at its inner end is tapered at 15<sup>a</sup> to form 55 the conical or taper part of the valve tip, and this part of the cavity is connected with the pouring cavity by means of a small cylindrical ingate 16. Each of the mold cavities is formed 60 at its outer end with an enlarged threaded section 15<sup>b</sup> designed to receive a screw plug 17 which serves as an abutment for the outer end of the valve shank and prevents its outward displacement by the centrifugal force of the molten metal. The threaded plugs 17 can easily be turned to adjust 65 their position according to the length of the valve shank. To avoid the necessity of screwing the plugs in each time the mold is assembled, said plugs can be carried in one or the other of the two main parts of the mold so that its adjusted 70 position is not disturbed when the mold sections 75

are separated. Thus, in the construction illustrated, the bottom part 8 of the mold has its upper face formed with a depression or annular rabbet 17<sup>a</sup> and the top part 9 of the mold is formed with a corresponding annular downward extension so that the screw plugs have more than half of their peripheral surfaces embraced by the top part 9 of the mold and are therefore not separated from said mold part when it is removed from the bottom part of the mold.

5 10 A guard casing 18 having its bottom side open and its top side formed with a central aperture 18<sup>a</sup> is adapted to be detachably mounted on the top of the casing or frame of the motor 13 so as to substantially enclose the mold and stop flying molten metal that might escape from the pouring cavity 14 when the mold is rotated.

In operating the mold, with the top part 15 removed, the prepared valve shanks 1 are placed in position on the bottom part 8 of the 20 mold. The top part 9 is then placed in position on said bottom part and secured by nuts 11. In the initial operation of the mold, the screw plugs 17 are then inserted until their inner ends press the valve shanks as far inward as the mold cavity 25 will permit whereupon the screws 17 are backed off slightly to provide a slight clearance between them and the valve shanks.

The form of the valve shank when it is placed in the mold is shown by the full lines in Fig. 4 except at the bevel or taper 4 where the form of the shank taper is represented by the dot-and-dash lines. Furthermore the taper part 15<sup>a</sup> of the mold cavities also correspond to the dot-and-dash lines in Fig. 4 of the drawings, thus providing for 30 metal to be removed in finishing the tip end of the valve.

The mold is preferably heated to some extent before pouring the molten metal into it. Accordingly when the mold parts have been assembled 40 with the valve shanks therein the entire structure including the shanks is heated to a temperature of about 750° F. This can be done with a suitable torch, but I prefer to do it by detaching the mold from the drive shaft 12 and placing it in 45 an oven which is maintained at the desired temperature. When the mold has been heated the guard or cover 18 is placed in position, the motor started and the molten stellite or other metal is poured through the aperture 18<sup>a</sup> into the pouring 50 cavity 14. In the use of stellite I pour the molten metal at a temperature of about 3200° F.

When the molten metal enters the pouring cavity 14 the rotation of the mold, for which I have found a speed of about 2200 R. P. M. suitable, sets up a rotary movement of the molten metal and the resultant centrifugal force feeds the molten metal under corresponding pressure through the small ingate 16 into the casting cavity formed by the mold proper and the inner ends of 60 the valve shanks 15. Although the entering molten metal is strongly chilled by the walls of the ingate and casting cavities, the latter are always effectively filled because of the strong centrifugal force to which the molten metal is subjected. However, when the molten metal sets and cools, the combined effect of the crystallization shrinkage and the contraction due to cooling is to cause a substantial contraction of the cast metal. While this has the effect of forming the 65 voids illustrated in Fig. 4 and above referred to, it also results in the drawing of the tapered shoulders of the cast tip strongly against the opposing shoulders of the valve shank so that the tip and shank are powerfully clamped together. The 70 75

contraction also usually has the effect of rupturing the cast metal in the ingate where it joins the larger body of the cast metal remaining in the pouring cavity 14. Thus, when the mold is dis-  
5 assembled by removing the top part 9, the valves are ordinarily already separated from the sprue in the pouring cavity 14 and can be individually lifted or shaken out.

The valves, on removal from the mold, have the  
10 form shown by the dot-and-dash lines in Fig. 4 and the next step in the manufacture of the valve is the grinding away of the excess metal of the tip to reduce it to the form shown by full lines in Fig. 4. In grinding the tip 5 to the finished  
15 conical or taper form shown in full lines, a corresponding amount of metal at the taper 4 of the shank 1 is simultaneously removed.

On referring to Fig. 4, it will be observed that it is necessary to remove but a small amount of the  
20 cast stellite in the grinding operation. This is an important consideration because the strong chilling effect on the outer layer of the casting produces a dense, fine-grained structure free from porosity and, by so forming the cast tip that it is  
25 not necessary in the finishing operation to cut through this outer fine-grained layer of the casting, I avoid exposing the porous structure which tends to exist in the deeper, less chilled layers of the casting. In other words, I thus secure valve  
30 tips with smooth surface and avoid losses which would occur due to the exposure of porous metal if the above mentioned conditions were not secured. As shown by Fig. 4, the grinding operation penetrates to the axis of the ingate metal at  
35 the valve point. Consequently the provision of a relatively small ingate for the molten metal is essential to insure chilling and the resulting dense, fine-grained structure of the metal throughout the ingate part of the casting. Hence,  
40 with the small ingate and the heavy chilling action, the strong centrifugal force to which the molten metal is subjected plays an important part in insuring the complete filling of the mold cavity and the avoidance of imperfect castings.

45 The contraction of the stem 5<sup>b</sup> of the tip 5, which is relied upon to rigidly secure the tip to the shank of the valve, sets up a relatively high stress in the stem part of the cast tip and it is therefore important to avoid porosity in this  
50 stem part in order to avoid fracture thereof. I prevent such porosity in the stem 5<sup>b</sup> of the tip as well as in the ingate to the cavity by suitable design of the casting cavity. It will be observed that the shape of the cavity is made such  
55 that the cast valve tip has the largest mass of its constituent metal in the region between the ingate and the stem 5<sup>b</sup>. Consequently, in casting the valve tip the interior part of this larger mass of metal in the intermediate zone remains molten longer than the metal in the stem 5<sup>b</sup> and the metal which is to form the conical seat-engaging surface of the tip (including the metal in the innermost part of the ingate), with the result that crystallization shrinkage of the earlier setting  
60 metal in these two regions is compensated for with metal drawn from the interior mass of metal still remaining in the molten state in the enlarged intermediate section of the casting. This usually results in some porosity in the interior region of the tip between the stem 5<sup>b</sup> and the conical seat-engaging walls of the tip, but such inferior porosity is not exposed by the relatively shallow finishing operation on the valve and does not reach the stem 5<sup>b</sup> and so does no harm.

70 It is to be observed, in connection with valves

of the type shown in Figs. 1, 2, 3 and 4, that since the shrinkage of a metal such as stellite on casting is quite considerable, the internal stresses set up are correspondingly large and this must be borne in mind in designing the valve and stresses great enough to rupture the metal avoided. In Fig. 4, for example, the length of the neck section 5<sup>b</sup> of the tip 5 between the latter's taper shoulders 6 and 7 is so proportioned that the contraction of the tip on casting shall be just  
10 sufficient to effect the desired clamping action between the tip and the shank without setting up unduly large stresses in the metal of the tip. The valve shown in Fig. 3 and presently to be referred to is to be designed with similar precaution.  
15

While the type of valve construction shown in Fig. 4 is one that I have found especially satisfactory in the production of needle valves, other forms of construction can be used in carrying out my invention. In Fig. 5 I have shown a form of valve having the same general structural and functional characteristics as the valve shown in Fig. 4. Here, as in Fig. 4, the full lines show the finished construction and the dot-and-dash lines  
20 show the valve as it is taken from the mold after casting on the valve tip. In this last construction the shank 18 is machined out at one end to form a cavity with walls that are undercut with relation to the end opening of the cavity, said  
25 walls comprising a short taper at 19<sup>a</sup> and a long taper at 19<sup>b</sup>. The outer surface at this same end of the shank is formed with a bevel or taper 19<sup>c</sup>. Into this cavity of the shank is cast a tip 20 of stellite or other suitable metal. Obviously this  
30 can be done in a mold of the character above described. When the tip 20 shrinks, on casting, it tends to draw away from the walls of the shank cavity and become loose. To secure the tip tightly in the cavity, I place the valve shank in swaging dies and subject it to pressure to form the circular groove 19<sup>d</sup>. This forces the metal of the shank inward against the inner tapered end of the tip 20 and forces the tip outward against the inwardly tapered surfaces 19<sup>b</sup> of the shank  
35 thus detaining and rigidly securing the tip. After this swaging operation the valve is ready for the  
40 finishing grinding operation which effects the removal of excess metal on the outer conical surfaces of the valve represented by the dot-and-dash lines in Fig. 5.  
45

It will be seen that the principles involved in the constructions and the methods of production of the two forms of valve above described have much in common. In each case the construction of the valve is such that the cast tip is very rigidly and firmly secured to the shank by internal stresses that are set up in one or the other of the two valve parts. In the first form of valve the construction of the cast tip on casting sets up a strong internal tension in the tip so that the latter has its taper surfaces drawn against corresponding opposing surfaces of the shank, thereby producing a very strong clamping force. In the second valve the swaging of  
55 the shank 18 sets up a reaction between the taper surfaces of the cast tip and of the shank respectively, with corresponding tension in the metal of the shank which surrounds the tip. In making the valves, in each case, porosity of the  
60 cast metal forming the seat-engaging portions of the valve is avoided by the use of a suitably constructed ingate and by providing a relatively large mass of cast metal adjacent to the seat-engaging surfaces so that the crystallization shrinkage of  
65 70 75

the metal forming such surfaces is compensated for with molten metal drawn from the interior of the tip where resultant porosity does no harm.

The mold shown in Fig. 3 of the drawings is of the same general construction as that shown in Figs. 1 and 2 but presents some detail differences which in practice I have found advantageous. The mold consists of bottom and top parts 21, 22, respectively, formed with opposite radial recesses 21<sup>a</sup>, 22<sup>a</sup>, to receive the valve shanks, the top part being detachably secured to the bottom part by machine screws 23. The top part is provided with the undercut pouring opening 22<sup>b</sup> and the central top surface of the bottom part 21 is raised in convex form at 21<sup>b</sup>. Each of the radial grooves of the bottom part is supplied with a malleable metal stop pin 24 to position the outer end of the valve shanks when they are assembled in the mold. These stop pins can be slightly adjusted by bending them with a hammer or the like to secure the correct positioning of the valve shanks. The shank and cast tip parts of a valve are shown in section, the valve shank being designated by the numeral 25 and the tip part by 26. Here the stem part 26<sup>a</sup> of the tip has its diameter and length approximately the same as the diameter and length, respectively, of the ingate part 26<sup>b</sup>.

The mold shown in Fig. 3 is operated in substantially the same manner as the mold shown in Figs. 1 and 2 so that its operation need not be described. I have found in practice that the convex surface 21<sup>b</sup> of the mold tends to prevent the sprue metal from sticking to the mold. I have also found that by making the stem 26<sup>a</sup> of the valve tip of approximately the same diameter and length as the ingate metal 26<sup>b</sup> the porosity of the cast tip is limited more completely or perfectly to the central interior region 40 of the main mass of the tip metal so that there is a more perfect avoidance of defective valves due either to outcropping of porosity on the seat-engaging surfaces of the finished valve or to encroachment of porosity upon the stem section 45 of the tip with resultant weakening and breakage of the stem incident to the tension set up in it on the freezing of the metal.

Where large numbers of valves are to be produced of given length it is obvious that the use of stop pins 24 in lieu of adjustable screws considerably reduces the cost of the mold and provides a construction that is equally satisfactory in operation.

By the use of my improved method of producing composite valves, economies are realized in production which are quite notable in comparison with other methods known to me. Perhaps the most important economy is due to the minimizing of defectives resulting either from porosity or from fracture of the cast tip part of the valve. Another economy which results from the casting of the hard metal tip on the shank with interlocking relation, is due to the fact that metals suitable for such casting purposes are available at a much lower price than similar metal purchased in definite forms or shapes. This is notably true in the case of the alloy stellite. By the use of mold apparatus of the character herein disclosed and by following procedures such as have been described, my method can be carried out rapidly and precisely with a minimum amount of labor and with the production of a highly uniform product, all of which factors contribute to economy of production.

While I have described specific forms of valve construction and of mold apparatus and pre-

ferred procedure, it will be understood that the carrying out of the method is subject to variation in all these respects within the bounds of the appended claims.

What I claim is:

1. A method of making a composite valve comprising a metal shank and a seat-engaging head of hard, wear-resisting cast metal subject to porosity when cast, the said method consisting in placing the shank in a metal mold with a portion of the shank forming part of the wall of a casting cavity which approximates the form of the cast metal head part of the finished valve; pouring the molten casting metal into the mold cavity to form the valve head; compensating for crystallization shrinkage of the metal forming the seat-engaging portion of the head; and thereafter reducing the cast part of the valve to finished form. 20

2. A method of making a composite needle valve comprising a metal shank and a conical seat-engaging tip of hard, wear-resisting cast metal subject to porosity when cast, the said method consisting in placing the shank in a metal mold with one end of the shank forming part of the wall of a casting cavity which approximates the form of the cast metal tip part of the finished valve and which has a restricted ingate passage leading axially into the conical end of the cavity; forcing molten casting metal into the casting cavity through said ingate passage to form the valve tip; compensating for crystallization shrinkage of the metal forming the conical sides of the finished valve tip with molten metal from the interior of the tip; and thereafter reducing the cast part of the valve to finished form. 30

3. A method of making a composite needle valve comprising a metal shank and a conical seat-engaging tip of hard, wear-resisting cast metal subject to porosity when cast, the said method consisting in placing the shank in a metal mold with one end of the shank forming part of the wall of a casting cavity which approximates the form of the cast metal tip part of the finished valve and which has a restricted ingate passage leading axially into the conical end of the cavity; pouring molten casting metal into the mold and simultaneously rotating the mold to introduce the molten metal through the ingate passage by centrifugal force to form the valve tip; compensating for crystallization shrinkage of the metal forming the conical sides of the finished valve tip with molten metal from the interior of the tip; and thereafter reducing the cast part of the valve to finished form. 40

4. A method of making a composite needle valve comprising a metal shank and a conical seat-engaging tip of cast metal, the said method consisting in placing the shank in a metal mold with one end of the shank forming part of the wall of a casting cavity which approximates the form of the cast metal tip part of the finished valve and which has a restricted ingate passage leading axially into the conical end of the cavity; pouring molten casting metal into the mold and simultaneously rotating the mold to introduce the molten metal through the ingate passage by centrifugal force to fill the cavity and form the valve tip; and thereafter reducing the cast part of the valve to finished form. 60

5. A method of making a composite needle valve comprising a metal shank and a conical seat-engaging tip of cast metal, the said method con- 70

- sisting in forming the shank with an undercut portion at one end; placing the shank in a metal mold with the undercut end of the shank forming part of the wall of a casting cavity which approximates the form of the cast metal tip part of the finished valve and which has a restricted ingate passage leading axially into the conical end of the cavity; pouring molten casting metal into the mold and simultaneously rotating the mold to introduce the molten metal through the ingate passage by centrifugal force to fill the cavity and form the valve tip; subjecting the shank to a swaging operation to effect a rigid interlocking connection between the shank and tip; and thereafter reducing the cast part of the valve to finished form. 5
6. A method of making a composite needle valve comprising a metal shank and a conical seat-engaging tip of cast metal, the said method consisting in forming the shank with an undercut axial bore in one end; placing the shank in a metal mold with its said end forming part of the wall of a casting cavity which approximates the form of the cast metal tip part of the finished valve and which has a restricted ingate passage leading axially into the conical end of the cavity; pouring molten casting metal into the mold and simultaneously rotating the mold to introduce the molten metal through the ingate passage by centrifugal force to fill the cavity and form the cast tip of the valve with an interlocking connection with the shank; and thereafter reducing the cast part of the valve to finished form. 10
7. A method of making a composite needle valve comprising a metal shank and a conical seat-engaging tip of cast metal, the said method consisting in forming the shank with an undercut portion at one end; placing the shank in a metal mold with the undercut end of the shank forming part of the wall of a casting cavity which approximates the form of the cast metal tip part of the finished valve and has a restricted ingate passage leading axially into its conical end and is shaped to afford in the casting operation a relatively large mass of molten metal adjacent to the conical cavity walls forming the seat-engaging part of the valve tip; pouring the molten metal into the mold and simultaneously rotating the mold to introduce the molten metal through the ingate passage by centrifugal force to fill the cavity and form the cast tip of the valve with an interlocking connection with the shank; and thereafter reducing the cast part of the valve to finished form. 15
8. A method of making a composite valve comprising a metal shank and a seat-engaging head of hard, wear-resisting cast metal subject to porosity when cast, the said method consisting in placing the shank in a metal mold with a portion of the shank forming part of the wall of a casting cavity which approximates the form of the cast metal head part of the finished valve; pouring the molten casting metal into the mold cavity to form the valve head; compensating for crystallization shrinkage of the metal forming the seat-engaging portion of the head with molten metal from the interior of the head; subjecting the shank to a swaging operation to effect a rigid interlocking connection between the shank and head; and thereafter reducing the cast part of the valve to finished form. 20
9. A method of making a composite needle valve comprising a metal shank and a conical seat-engaging tip of cast metal, the said method consisting in placing the shank in a metal mold with one end of the shank forming part of the wall of a casting cavity which approximates the form of the cast metal tip part of the finished valve and which has a restricted ingate passage leading axially into the conical end of the cavity; pouring molten casting metal into the mold and simultaneously rotating the mold to introduce the molten metal through the ingate passage by centrifugal force to fill the cavity and form the valve tip; subjecting the shank to a swaging operation to effect a rigid interlocking connection between the shank and tip; and thereafter reducing the cast part of the valve to finished form. 25
10. A method of making a composite needle valve comprising a metal shank and a conical seat-engaging tip of cast metal, the said method consisting in forming the shank at one end with an axially extending cavity having its side wall undercut in relation to its mouth; placing the shank in a metal mold with its cavity end forming part of the wall of a casting cavity which approximates the form of the cast metal tip part of the finished valve and which has a restricted ingate passage leading axially into the conical end of the cavity; pouring molten casting metal into the mold and simultaneously rotating the mold to introduce the molten metal through the ingate passage by centrifugal force to fill the cavity and form the valve tip; subjecting the shank to a swaging operation to effect a rigid interlocking connection between the shank and tip; and thereafter reducing the cast part of the valve to finished form. 30
11. A method of making a composite needle valve comprising a metal shank and a conical seat-engaging tip of cast metal, the said method consisting in forming the shank at one end with an axially extending cavity having its side wall undercut in relation to its mouth and with an annular shoulder surrounding the mouth of the cavity; placing the shank in a metal mold with the wall of the cavity and the said shoulder forming part of the wall of a casting cavity which approximates the form of the cast metal tip part of the finished valve and which has a restricted ingate passage leading axially into its conical end; pouring molten casting metal into the mold and simultaneously rotating the mold to introduce the molten metal through the ingate passage by centrifugal force to fill the cavity and form the cast tip of the valve with an interlocking connection with the shank; and thereafter reducing the cast part of the valve to finished form. 35
12. A method of making a composite needle valve comprising a metal shank and a conical seat-engaging tip of cast metal, the said method consisting in forming the shank at one end with an axially extending bore and with two annular shoulders surrounding the side wall of the bore and facing away from each other; placing the shank in a metal mold with the wall of its bore and the said shoulders forming part of the wall of a casting cavity which approximates the form of the cast metal tip part of the finished valve and which has a restricted ingate passage leading axially into the conical end of the cavity; pouring molten casting metal into the mold and simultaneously rotating the mold to introduce the molten metal through the ingate passage by centrifugal force to fill the cavity and form the cast tip of the valve with an interlocking connection with the shank; and thereafter reducing the cast part of the valve to finished form. 40
- 75